

1

2

3,164,553

## PROCESS OF TREATING SYNTHETIC LUBRICATING OILS WITH UREA

Robert A. Cupper, Ridgefield, Conn., and Carl A. Wolf, Jr., New York, N.Y., assignors to Union Carbide Corporation, a corporation of New York  
No Drawing. Filed Dec. 16, 1960, Ser. No. 76,118  
17 Claims. (Cl. 252—51.5)

This invention relates to lubricating oil compositions of good viscosity and anti-sludging characteristics, and more particularly, to the improvement of providing lubricating oil compositions having improved anti-corrosive action on metals.

A wide variety of ester type synthetic lubricants are known in the art as being useful as lubricants for aircraft turbine engines having high compression ratios and increased power outputs, such as turbojets and turboprop combustion engines. The use of synthetic esters has made it possible to extend the range of ambient temperatures encountered and allow increased engine operating temperatures.

However, the synthetic esters commonly employed as lubricants suffer from the disadvantage of being corrosive towards metal, particularly at high temperatures. It is immediately apparent that much damage can occur to vital parts of an engine by the use of lubricants which have corrosive action towards metal.

Accordingly, it is the object of this invention to provide lubricating oil compositions offering increased corrosion protection towards metal.

It has now been found that the anti-corrosion characteristics of synthetic esters can be markedly improved by treating said esters with urea.

The novel lubricants of this invention are prepared by adding from 0.05 to 1.0 percent by weight of urea to a base fluid, or mixtures of base fluids, and heating to a temperature within the range of 125 to 250° C. The preferred temperature range is from 180 to 210° C. and the preferred concentration of urea is 0.1 to 0.5 percent by weight.

If the base fluid being treated has a tendency to decompose, it is preferred to conduct the heating at reduced pressures or under an inert atmosphere or under both an inert atmosphere and reduced pressure.

The term base fluid, as used in the specification and the claims, refers to synthetic esters including diesters, polyesters and polyglycol derivatives, which are used as bases for lubricants.

After the base fluids have been heated for a period of time, which varies with the particular base fluid, but is usually from 10 to 60 minutes, they are subjected to a conventional filtration step to remove precipitated materials.

The synthetic base fluids to which the urea is added are well known in the art. It is to be understood that the novel lubricants of this invention contain a base fluid or mixtures of base fluids which are conventional. The instant invention does not reside in the particular base fluids but rather in the treatment of conventional base fluids with urea to obtain lubricants having superior anti-corrosive action on metals, particularly copper and lead.

The base fluids which can be treated with urea include:

(A) Diesters of aliphatic dicarboxylic acids which correspond to the formula:



wherein  $n$  is an integer from 2 to 18, each  $R^2$  represents

alkyl or cycloalkyl radicals having from about 5 to 24 carbon atoms and preferably from about 5 to 18 carbon atoms, and  $R'$  represents hydrogen or alkyl groups having from 1 to 4 carbon atoms. The dicarboxylic acids may be substituted, such as, for example, 3-methyl glutaric acid, to obtain lower viscosities at low temperatures so long as this substitution is consistent with the need for obtaining a low freezing point. Specific examples of organic dicarboxylic acids from which the esters may be derived are suberic, adipic, brassilic, Japanic, sebacic, glutaric, azelaic, and pimelic acids, as well as mixtures of these acids. The preferred acids are azelaic, adipic, and sebacic acids.

The alcohols used to form the diester of the acid may be branched chain or straight chain, saturated or unsaturated, aliphatic or cycloaliphatic alcohols. Typical alcohols which may be employed include 2-ethylhexyl alcohol, isoctyl alcohol, isodecyl alcohol, 2-ethylbutyl alcohol, cetyl alcohol, n-octyl alcohol, amyl alcohol, oleyl alcohol, 2-butyloctyl alcohol, methyl and dimethylcyclohexanol, and the "Oxo" alcohols, such as the mixed branched chain nonanols, prepared from the reaction of carbon monoxide and hydrogen upon olefins which normally have a branched chain structure. Mixtures of alcohols can also be used such as a mixture of 2-ethylhexyl and isodecyl alcohol.

Representative synthetic diester lubricants which can be employed in conjunction with this invention include

30 di-(2-ethylhexyl)sebacate,  
di-(2-ethylhexyl)azelate,  
di[mixed-(2-ethylhexyl, isodecyl)]azelate,  
di-(isoctyl)azelate,  
di-(1-methylcyclohexylmethyl)sebacate,  
35 di-(2-ethylhexyl, decyl)azelate,  
di-(2-ethylhexyl-2-propylheptyl)azelate,  
di-(2,2,4-trimethylpentyl)sebacate,  
di-(2-methylpentyl, decyl)azelate,  
40 di-(1-ethylpropyl)adipate,  
di-(3-methylbutyl)adipate,  
di-(1,3-dimethylbutyl)adipate,  
di-(2-ethylbutyl)adipate,  
di-(2-ethylhexyl)adipate,  
45 di-(isoctyl)adipate,  
di-(undecyl)adipate,  
di-(tetradecyl)adipate,  
di-(heptadecyl)adipate,  
di-(2,2,4-trimethylpentyl)adipate,  
50 di-(1-methylcyclohexylmethyl)adipate,  
di-(1-ethylpropyl)-azelate,  
di-(3-methylbutyl)azelate,  
di-(2-ethylbutyl)azelate,  
di-(1-ethylpropyl)sebacate,  
55 di-(3-methylbutyl)sebacate,  
di-(1,3-dimethylbutyl)sebacate,  
di-(2-ethylbutyl)sebacate,  
di-(2-ethylhexyl)sebacate,  
di-(2-(2'-ethylbutoxy)ethyl)sebacate,  
60 di-(undecyl)sebacate,  
di-(tetradecyl)sebacate,  
di-(heptadecyl)sebacate,  
di-(2-ethylhexyl)glutarate,  
di-(undecyl)glutarate,  
di-(tetradecyl)glutarate, and the like.

(B) Esters of aromatic acids which correspond to the general formula:



70 wherein  $Z$  represents a phenyl radical or a naphthyl radical,  $n$  represents an integer from 2-4 and  $R^2$  has the same meaning as previously described.

Examples of acids from which the esters can be prepared include phthalic terephthalic, pyromellitic, naphthalene-1,4-dicarboxylic acid, etc. The alcohols which are reacted with the aromatic acids are the same as those mentioned under A.

(C) Complex glycol centered esters having the general formula:



wherein  $n$  represents a number from 3-51,  $\text{R}^2$  represents alkyl or cycloalkyl radicals having from 4 to 24 carbon atoms and  $\text{R}^3$  represents hydrogen, methyl or ethyl.

Examples of the above esters include 3-methyl-1,5-pentanediol diisododecanoate and hexamethylene 1,6-glycol-diisooctanoate.

(D) Complex glycol centered esters containing recurring ether linkages represented by the formula:



wherein  $\text{R}^2$  represents alkyl or cycloalkyl radicals having from 4 to 24 carbon atoms,  $\text{R}^4$  represents hydrogen, methyl or ethyl and  $n, m$  and  $X$  represent an integer from 1-25.

Examples of the above esters include dipropylene glycol dipelargonate, polyethylene glycol 200 di-valerate and polypropylene glycol 425 di-2-ethyl hexanoate.

(E) Polyol monobasic acid esters corresponding to the formula:



wherein  $n$  is an integer from 3-4 and  $\text{R}^5$  represents an alkyl group having from 0-8 carbon atoms, with the proviso that when  $\text{R}^5$  is 0,  $n$  is 4, and  $m$  is an integer from 0 to 18.

Examples of alcohols which are reacted with aliphatic monocarboxylic acids include trimethylol ethane, trimethylol propane and pentaerythritol.

It is to be understood that the above classes of base fluids are representative of art recognized fluids and are merely illustrative of some of the base fluids useful in this invention. The complex esters have been described in the art as well as in U.S. Patents 2,575,195; 2,575,196; and 2,703,811.

(F) Alkyl terminated polyesters: These are complex polyesters prepared from polyhydric alcohols and polybasic acids wherein reactive carboxyl or hydroxyl groups are terminated by reaction with either monofunctional alcohols or acids. These esters are known in the art and described in U.S. Patent 2,705,724. The disclosure of said patent is incorporated by reference into this application.

(G) Non-terminated or hydroxyl terminated polyesters: This class of compounds refers to those polyesters having free hydroxyl groups in the polymer chain which are not blocked or terminated by reaction with monofunctional or polyfunctional compounds. These compounds are known in the art and can be prepared by reacting a dibasic acid with a glycol or alkane diol as disclosed in U.S. Patent 2,929,786 or by reacting a dibasic acid with mixtures of polypropylene glycol and a 1,3-alkanediol as disclosed in copending application Serial No. 718,971.

(H) Polyalkylene glycol derivatives: These compounds can be represented by the formula:



wherein  $\text{R}^6$  represents hydrogen or an alkyl radical having from 1-12 carbon atoms,  $\text{R}^4$  represents hydrogen or an alkyl radical having from 1-2 carbon atoms and each of  $n, m$  and  $X$  represent a positive integer from 1-25.

The integers  $m$  and  $n$  can be varied so as to provide homo- and heteropolymers, i.e., polyoxyethylene glycols, polyoxypropylene glycols, mixed poly(oxyethylene-oxypropylene) glycols and also the mono- and diethers of the above.

This class of compounds is well known in the art and the individual members of this class can be made in a variety of ways. Illustrative of the above class of compounds, as well as methods for the preparation of individual members are U.S. Patents 2,293,868; 2,425,755; 2,425,845; 2,448,664; 2,520,611 and 2,520,612.

The preferred compounds in this class are the mono-butyl ethers.

It is to be understood that this invention relates to the treatment of base fluids in a novel manner and not to the particular base fluids employed. Thus, the above classes of base fluids (A to H) are representative of base fluids which can be treated according to the novel process of this invention. It is also within the scope of this invention to treat mixtures of base fluids which have been designated by A to H.

It is to be understood that the novel lubricants of this invention can contain conventional additives, e.g., viscosity index improvers, detergents and antioxidants, as is customary in this art. The preferred antioxidants are amine compounds such as phenothiazine, N-phenyl-beta-naphthylamine, N-phenyl-alpha-naphthylamine, and phenolic compounds such as di-tert-butyl para-cresol and butylated hydroxyanisole.

The following table depicts the critical specifications of a gas turbine lubricant and is based upon U.S. Specification Mil-L-7808C. Somewhat similar specifications are required for turboprop lubricants as described by EMS 35E of the Allison Division of General Motors Corporation and Specification D. Eng. R.D. 2487 (Second Issue) of the British Ministry of Supply.

TABLE I.—CRITICAL GAS TURBINE AIRCRAFT LUBRICANT SPECIFICATIONS

| Corrosion and Oxidation                           | Standard 347° F. Test | 352° F. Test   |
|---------------------------------------------------|-----------------------|----------------|
| Weight Change, mg./sq. cm.:                       |                       |                |
| Copper.....                                       | ±0.4                  | ±0.4           |
| Magnesium.....                                    | ±0.2                  | .....          |
| Aluminum.....                                     | ±0.2                  | .....          |
| Steel.....                                        | ±0.2                  | ±0.2           |
| Silver.....                                       | ±0.2                  | .....          |
| Lead.....                                         | .....                 | ±1.0           |
| Viscosity Change, 100° F., percent.....           | -5 to +15             | -5 to +15      |
| Neut. No. Increase, mg. KOH/g.....                | 2.0                   | 2.0            |
| SOD lead corrosion, 1 hr. at 325° F., mg./sq. in. |                       | 6.0 (max).     |
| Corrosion, 50 hr. at 450° F., mg./sq. in.         |                       |                |
| Copper.....                                       | .....                 | 3.0 (max).     |
| Silver.....                                       | .....                 | 3.0 (max.).    |
| Panel coking, 8 hours at 600° F.                  |                       | 80 mg. (max.). |

*Test methods.*—The 352° F. corrosion and oxidation test was employed as the primary tool to evaluate urea-treated fluids. The 352° F. test, designed to simulate the standard military corrosion and oxidation test (791.5308.4) was simplified by eliminating aluminum, magnesium, and silver metals, and adding a lead specimen. Steel and copper coupons are used in both tests. The 352° F. test consists of maintaining the test fluid at test temperature in the presence of the steel, copper, and lead specimens for 72 hours while purging with air at the

rate of 5 liters per hour. At the completion of the test, the fluid is observed for the separation of insolubles and for viscosity change. The weight change of the metal specimens is also determined.

The SOD (Standard Oil Development Company) lead corrosion test was also used. This is the standard test procedure employed by the military for evaluating the tendency of gas turbine lubricants to corrode lead. The Allison Division (General Motors Corporation) aircraft gas turbine lubricant specifications include the SOD lead corrosion test. This test consists in rotating copper and lead (weighed) specimens for one hour in the test fluid which is maintained at 325° F. During the test, air is passed through the fluid at a rate of 57 liters per hour. The weight change of the lead specimen, in milligrams per square inch, is determined. At the present time, all lubricant specifications containing this test allow a maximum lead corrosion value of 6.0 milligrams per square

duced the lead corrosion rate from 11.5 milligrams per square inch to 0.19 milligram per square inch.

*Example 3*

5 A sample of tri-(2-ethylhexyl) phosphate ("Flexol" TOF) was treated by adding 0.5 percent urea to the dried fluid and agitating at 160°-165° F. for 5 minutes. This fluid, as well as an untreated sample from the same batch, after addition of 0.5 percent phenothiazine, were exposed to the 352° F. corrosion and oxidation test. Copper and lead corrosion rates are shown below.

| 15                        |  | Weight Loss, mg./cm. <sup>2</sup> |      |
|---------------------------|--|-----------------------------------|------|
|                           |  | Copper                            | Lead |
| Before Treatment.....     |  | 26.0                              | 63.3 |
| After Urea Treatment..... |  | 3.1                               | 18.1 |

TABLE II.—TREATMENT OF ALIPHATIC DIBASIC ACID ESTERS WITH UREA

[Antioxidant=0.5% (wt.) purified phenothiazine]

| Base Fluid.....                                                    | C <sub>8</sub> -C <sub>10</sub> -Az. <sup>2</sup> | C <sub>8</sub> -C <sub>10</sub> -Az. | C <sub>8</sub> -C <sub>10</sub> -Az. | C <sub>8</sub> -C <sub>10</sub> -Az. | C <sub>8</sub> -C <sub>10</sub> -Az. | C <sub>8</sub> -Ad <sup>3</sup> | C <sub>8</sub> -Ad   |
|--------------------------------------------------------------------|---------------------------------------------------|--------------------------------------|--------------------------------------|--------------------------------------|--------------------------------------|---------------------------------|----------------------|
| Treatment <sup>1</sup> .....                                       | None                                              | 0.1% Urea at 180° C.                 | 0.25% Urea at 180° C.                | 1.0% Urea at 180° C.                 | 0.5% Urea 195-205° C.                | None                            | 0.5% Urea at 180° C. |
| 352° F. Corrosion-Oxidation: Viscosity Change at 100° F., Percent. | +4.5.....                                         | +4.7.....                            | +3.9.....                            | +3.5.....                            | +1.9.....                            |                                 |                      |
| Insolubles Formed.....                                             | Moderate.....                                     | Moderate.....                        | Moderate.....                        | Moderate.....                        | Small.....                           |                                 |                      |
| Appearance of Metals:                                              |                                                   |                                      |                                      |                                      |                                      |                                 |                      |
| Steel.....                                                         | Brown-Bronze.....                                 | Brown-Bronze.....                    | Steel-Bronze.....                    | Steel-Bronze.....                    | Shiny-Gray.....                      |                                 |                      |
| Copper.....                                                        | Dull Brown.....                                   | Dull Steel-Copper.....               | Dull Copper.....                     | Dull Copper.....                     | Dull, Red-Orange.....                |                                 |                      |
| Lead.....                                                          | Gray-Black.....                                   | Dull Gray.....                       | Dull Gray.....                       | Dull Gray.....                       | Dull, Gray-Black.....                |                                 |                      |
| Metal Weight Change, mg./cm. <sup>2</sup> :                        |                                                   |                                      |                                      |                                      |                                      |                                 |                      |
| Steel.....                                                         | +0.04.....                                        | +0.03.....                           | +0.05.....                           | -0.07.....                           | Nil.....                             |                                 |                      |
| Copper.....                                                        | -0.08.....                                        | -0.08.....                           | -0.14.....                           | -0.23.....                           | +0.03.....                           |                                 |                      |
| Lead.....                                                          | -1.6.....                                         | -0.16.....                           | -0.11.....                           | -0.86.....                           | -0.09.....                           |                                 |                      |
| SOD Lead Corrosion, mg./in. <sup>2</sup> .....                     | -2.0.....                                         |                                      |                                      |                                      | -0.19.....                           | -11.5.....                      | -0.19.....           |

<sup>1</sup> Treatment consisted in thoroughly mixing the urea with the base fluid with mechanical agitation and nitrogen purging for ½ hour at the temperature indicated.

<sup>2</sup> Di-(2-ethylhexyl, isodecyl)azelate.

<sup>3</sup> Di(2-ethylhexyl)adipate.

inch. Values under 1.0 milligram per square inch are highly desirable.

The following examples illustrate the novel lubricants of this invention.

*Example 1*

A sample of refined di-(2-ethylhexyl, isodecyl)azelate, containing 0.5 percent phenothiazine as an antioxidant, was tested in the 352° F. corrosion and oxidation test. The lead corrosion rate was found to be 1.6 milligrams per square centimeter. Separate portions of this diester were then treated with 0.1 to 0.25, and 1.0 percent urea at 180° C. Another portion was treated with 0.5 percent urea at 195-205° C. These treated samples were then tested in the 352° F. corrosion oxidation test after the addition of 0.5 percent phenothiazine. The data in Table II illustrate the marked decrease in the lead corrosion rate resulting from the urea treatment. The optimum urea concentration is about 0.5 percent.

The untreated sample and a sample treated with 0.5 percent urea were also evaluated in the SOD lead corrosion test. Phenothiazine was again used as the antioxidant. Again a substantial reduction in the lead corrosion rate was observed (Table II).

*Example 2*

A sample of refined di-2-ethylhexyl adipate was treated with 0.5 percent urea at 180° C. After the addition of 0.5 percent of phenothiazine, both the treated and untreated samples were tested in the SOD lead corrosion test. The data in Table II shows that urea treatment re-

45 Di-(2-ethylhexyl, isodecyl)azelate was prepared by tetraethyl orthotitanate catalysis as a residue product. Before stripping off the excess 2-ethylhexanol employed during the esterification, the crude mixture was mixed thoroughly in the presence of 0.5 percent urea for one-half hour at 180° C., while purging with nitrogen. The mixture was refined by contact filtration with diatomaceous earth and stripped. In practice, the filtration and stripping operations are sometimes reversed. Another portion of the crude diester was treated with 0.05 percent melamine by mixing for 15 minutes at 110°-120° C., and contact filtering with diatomaceous earth. Comparative results of the two treatments are shown below:

| 60                    |  | Weight change, mg./cm. <sup>2</sup> |            |
|-----------------------|--|-------------------------------------|------------|
|                       |  | Copper                              | Lead       |
| Melamine Treated..... |  | Nil.....                            | -0.11..... |
| Urea Treated.....     |  | +0.03.....                          | -0.03..... |

*Example 5*

A sample of polypropylene glycol 425 azelate was treated with urea according to the procedures outlined in Table III. The 352° F. corrosion and oxidation tests 70 results obtained with lubricants containing the treated polyesters are compared with results for blends containing untreated and melamine-treated polyesters. The improvement in lead corrosion as a result of urea treatment is obvious. On the basis of these experiments, the optimum treating temperature appears to be about 180° C.

TABLE III.—TREATMENT OF POLYESTERS WITH UREA

[352° F. corrosion and oxidation tests. Test fluid composition—80.0% (wt.) di-(2-ethylhexyl, isodecyl)azelate. 19.5% (wt.) 186-11 polypropylene glycol 425 azelate, 0.5% Purified Phenothiazine]

|                                             | Polypropylene Glycol 425 Azelate |                        |                              |                              |                        |                        |
|---------------------------------------------|----------------------------------|------------------------|------------------------------|------------------------------|------------------------|------------------------|
|                                             | 186-11 <sup>1</sup>              | 186-11R-1 <sup>2</sup> | 186-11U.5 <sup>3</sup> (120) | 186-11U.5 <sup>4</sup> (180) | 186-11U.1 <sup>5</sup> | 186-11U.5 <sup>6</sup> |
| Viscosity Change at 100° F., Percent.       | +2.0                             | +2.2                   | +3.1                         | -2.2                         | -0.34                  | -1.2                   |
| Insolubles Formed                           | None                             | None                   | Small                        | Slight                       | None                   | Slight                 |
| Appearance of Metals:                       |                                  |                        |                              |                              |                        |                        |
| Steel                                       | Brown-Bronze                     | Brown-Bronze           | Brown-Bronze                 | Brown-Bronze                 | Brown-Bronze           | Brown-Bronze           |
| Copper                                      | Pale, Pink-Copper                | Bright, Light Copper   | Brown-Copper                 | Brown-Copper                 | Steel-Copper           | Pale                   |
| Lead                                        | Gray-Black                       | Gray-Black             | Brown-Gray                   | Light Gray                   | Blue-Gray              | Dull Gray              |
| Metal Weight Change, mg./cm. <sup>2</sup> : |                                  |                        |                              |                              |                        |                        |
| Steel                                       | Nil                              | Nil                    | -0.019                       | Nil                          | -0.013                 | +0.05                  |
| Copper                                      | -0.24                            | -0.084                 | -0.21                        | -0.273                       | -0.273                 | -0.169                 |
| Lead                                        | -1.45                            | -1.1                   | -0.47                        | -0.06                        | -0.05                  | -0.39                  |

<sup>1</sup> Polypropylene Glycol 425 Azelate prepared from a 1.18:1.0 mole ratio of Polypropylene Glycol 425 and Emery Industries Emerox 1110 Azelaic acid.

<sup>2</sup> R-1=treatment with 0.05% (Wt.) melamine at 110-120° C.

<sup>3</sup> Treated with 0.5 percent (Wt.) urea for one-half hour at 120° C.

<sup>4</sup> Treated with 0.5 percent (Wt.) urea for one-half hour at 180° C.

<sup>5</sup> Treated with 0.1 percent (Wt.) urea for one-half hour at 240° C.

<sup>6</sup> Treated with 0.5 percent (Wt.) urea for one-half hour at 240° C.

#### Example 6

A sample of polypropylene glycol 425 azelate was prepared by a conventional esterification procedure using tetrabutyl orthotitanate as the catalyst and xylene as the azeotroping diluent. At the completion of the esterification reaction separate samples of the crude product were treated with urea as shown in Table IV.

30

#### Example 8

Two blends composed of 59.5 weight percent of di-(2-ethylhexyl isodecyl)azelate, 40 weight percent "Ucon" LB-625, and 0.5 weight percent N-phenyl-alpha-naphthylamine were evaluated in the SOD lead corrosion test. One blend contained the urea-treated "Ucon" LB-625 described in Example 7; the other was prepared from un-

TABLE IV.—TREATMENT OF CRUDE POLYPROPYLENE GLYCOL 425 AZELATE WITH UREA

Test fluid composition (percent by weight):  
 80.0% di-(2-ethylhexyl, isodecyl)azelate.  
 19.5% 186 polypropylene glycol 425 azelate.  
 0.5% Purified phenothiazine.

|                                                                    | Polypropylene Glycol 425 Azelate |                         |                         |
|--------------------------------------------------------------------|----------------------------------|-------------------------|-------------------------|
|                                                                    | 186-24 <sup>1</sup>              | 186-24-U-1 <sup>2</sup> | 186-24-U-2 <sup>3</sup> |
| 352° F. Corrosion-Oxidation: Viscosity Change at 100° F., percent. | -1.1                             | -2.2                    | -0.6                    |
| Insolubles Formed                                                  | Small                            | None                    | Small                   |
| Appearance of Metals:                                              |                                  |                         |                         |
| Steel                                                              | Brown-Bronze                     | Brown-Bronze            | Brown-Bronze            |
| Copper                                                             | Dull, Pale                       | Dull                    | Bright Gold Copper      |
| Lead                                                               | Dull, Gray-Black                 | Bright                  | Dull, Gray-Black        |
| Metal Weight Change, mg./cm. <sup>2</sup>                          |                                  |                         |                         |
| Steel                                                              | Nil                              | Nil                     | Nil                     |
| Copper                                                             | -0.18                            | -0.23                   | -0.09                   |
| Lead                                                               | -0.62                            | -0.07                   | -0.64                   |
| SOD Lead Corrosion, mg./in. <sup>2</sup>                           |                                  |                         |                         |

<sup>1</sup> Refined but not treated with urea.

<sup>2</sup> Treated with 0.5% urea for one-half hour at 180°-190° C.

<sup>3</sup> Treated with 0.5% urea for one-half hour at 230°-235° C.

#### Example 7

A sample of "Ucon" lubricant LB-625 (a polypropylene glycol monobutyl ether having a 100° F. SUS viscosity of 625) was treated by mixing thoroughly with 0.5 percent urea for one-half hour at 180° C. while purging with nitrogen. Samples of the treated and untreated fluid were tested in the SOD lead corrosion cell. The untreated fluid exhibited a lead weight loss of 2.0 milligrams per square inch, whereas the urea-treated sample showed a weight loss of only 0.15 milligram per square inch. One percent N-phenyl-alpha-naphthylamine was used as the antioxidant in each of these fluids.

65  
 70 treated "Ucon" LB-625. In the case of the untreated sample, a lead weight loss of 15.5 milligrams per square inch was obtained whereas a weight loss of only 5.6 milligrams per square inch was obtained for the treated sample.

#### Example 9

A lubricant blend composed of 81.0 weight percent of di-(2-ethylhexyl, isodecyl)azelate, and 19.0 percent polypropylene glycol 425 azelate was treated by mixing thoroughly with 0.5 percent urea for one-half hour at about 180°-190° C. This blend and a similar blend, which was not treated, were tested by means of the 352° F. corrosion and oxidation test. Data showing the improvement in

corrosion characteristics resulting from urea treatment are shown in Table V.

TABLE V.—UREA TREATMENT OF A DIESTER-POLYESTER BLEND

Test fluid composition:

99.5% Di-(2-ethylhexyl, isodecyl)-azelate.  
0.5% Polypropylene glycol 425 azelate.  
0.5% Purified Phenothiazine.

|                                             | Untreated Blend   | Urea Treated Blend <sup>1</sup> |
|---------------------------------------------|-------------------|---------------------------------|
| 352° F. Corrosion-Oxidation:                |                   |                                 |
| Viscosity Change at 100° F., percent.       | +7.4              | -1.3                            |
| Insolubles Formed                           | Small Amount      | None                            |
| Appearance of Metals:                       |                   |                                 |
| Steel                                       | Dull Brown-Bronze | Dark Brown-Bronze               |
| Copper                                      | Dull Silver       | Dull Brown-Copper               |
| Lead                                        | Dull Black        | Slightly Dull                   |
| Metal Weight Change, mg./cm. <sup>2</sup> : |                   |                                 |
| Steel                                       | Nil               | Nil                             |
| Copper                                      | -0.18             | -0.35                           |
| Lead                                        | -0.17             | -0.06                           |
| SOD Lead Corrosion, mg./in. <sup>2</sup>    | -5.4              | -0.21                           |

<sup>1</sup> Treated by mixing with 0.5% urea for one-half hour at 180°-190° C. while purging with nitrogen.

TABLE VI.—POLYOL CENTER ESTERS [Antioxidant—0.5% purified phenothiazine. 352° F. Corrosion Oxidation Test]

| Ester                             | Urea Treatment          |            |            | Viscosity Change at 100° F., Percent | Insolubles        | Metal Weight Change, mg./cm. <sup>2</sup> |        |       |
|-----------------------------------|-------------------------|------------|------------|--------------------------------------|-------------------|-------------------------------------------|--------|-------|
|                                   | Urea Conc., Wt. Percent | Temp., °C. | Time, Min. |                                      |                   | Steel                                     | Copper | Lead  |
| Diethylene Glycol Di-isodecanoate | None                    |            |            | +10.8                                | Moderate-Large... | +0.08                                     | -0.26  | -154  |
| Do.                               | 0.5                     | 220        | 30         | +6.2                                 | Moderate          | +0.05                                     | -0.02  | -24.1 |

### Example 10

(A) A sample of di-(isodecyl) adipate was treated with 0.1% by weight of urea at 200° C. for approximately 1/2 hour. The treatment was followed by contact filtration with diatomaceous earth to remove residues.

(B) A sample of di-(isoctyl) adipate was similarly treated.

(C) A sample of UCON Lubricant LB-1715 (a polyoxypropylene glycol monobutyl ether having a 100° F. SUS viscosity of 1715) was treated with 0.25% by weight of urea at 180° C. for approximately thirty minutes. The treatment was followed by contact filtration with diatomaceous earth to remove residues.

(D) A mixture was prepared consisting of:

30% by weight of A  
69% by weight of B  
1% by weight of C

The properties of this mixture are shown in Table VII and are contrasted with a mixture of the same components in the same proportions which have not been treated with urea.

TABLE VII.—ADIPATE DIESTER—POLYOXYPROPYLENE GLYCOLMONOBUTYL ETHER COMPOSITION

[352° F. corrosion-oxidation test. Antioxidant—0.5% phenothiazine]

|                                             | Fluid Made from Untreated Base Stocks | Fluid Made from Urea Treated Stocks |
|---------------------------------------------|---------------------------------------|-------------------------------------|
| Viscosity Change at 100° F., percent        | +1.7                                  | +2.7                                |
| Metal Weight Change, mg./cm. <sup>2</sup> : |                                       |                                     |
| Steel                                       | +0.03                                 | -0.01                               |
| Copper                                      | -0.20                                 | -0.22                               |
| Lead                                        | -4.6                                  | -1.4                                |

### Example 11

Samples of commercial diisooctyl adipate and diisodecyl adipate were found to have lead corrosion values of 33.0

and 31.9 milligrams per square inch respectively, when tested by the SOD lead corrosion procedure. After treatment of each of these diesters with 0.25 percent by weight of urea at 200° C., they exhibited lead corrosion values of 1.07 milligrams per square inch for the diisooctyl adipate and 0.54 milligram per square inch for the diisodecyl adipate.

As is evident from the foregoing examples and tables, the novel lubricants of this invention possess superior anti-corrosive properties.

What is claimed is:

1. A process which comprises contacting a synthetic lubricant base fluid with from 0.05 to 1.0 weight percent of urea, based on weight of said synthetic lubricant base fluid, at an elevated temperature, for a period of time sufficient to produce a synthetic lubricant having reduced corrosive tendencies to metals, said synthetic lubricant base fluid being of the group consisting of organic polyesters and organic ethers which are composed only of carbon, hydrogen, and oxygen.

2. The process of claim 1 wherein said process is carried out at a temperature in the range of from 125° C. to 250° C.

3. The process of claim 2 wherein the synthetic lubricant product is separated from solid material formed during said process.

4. A process for producing a synthetic lubricant which comprises the steps of contacting a synthetic lubricant base fluid with from 0.05 to 1.0 weight percent of urea, based on weight of said synthetic lubricant base fluid, at a temperature in the range of from 125° C. to 250° C., for a period of from 10 to 60 minutes, and thereafter recovering the synthetic lubricant thus produced, said synthetic lubricant base fluid being of the group consisting of organic polyesters and organic ethers which are composed only of carbon, hydrogen, and oxygen.

5. A process which comprises contacting a dialkyl diester of an alkanedioic acid with from 0.05 to 1.0 weight percent of urea, based on weight of said diester, at a temperature in the range of from 125° C. to 250° C. for a period of from 10 to 60 minutes, and thereafter recovering the said diester having reduced corrosive tendencies to metals which is thus produced, wherein the alkyl moieties of said diester have from 5 to 24 carbon atoms, and wherein the said alkanedioic acid has from 2 to 18 carbon atoms.

6. A process which comprises contacting a fully esterified alkyl ester of an aromatic polycarboxylic acid having from 2 to 4 carboxylic acid groups, with from 0.05 to 1.0 weight percent of urea, based upon weight of said ester, at a temperature in the range of from 125° C. to 250° C. for a period of from 10 to 60 minutes, and thereafter recovering the said ester having reduced corrosive tendencies to metals which is thus produced, wherein the alkyl moieties of said ester have from 5 to 24 carbon atoms.

7. A process which comprises contacting a fully esterified alkanoic ester of an alkanopolyol with from 0.05 to 1.0 weight percent of urea, based on weight of said ester, at a temperature in the range of from 125° C. to 250° C. for a period of from 10 to 60 minutes, and thereafter recovering the said ester having reduced corrosive tendencies toward metals which is thus produced, wherein the

alkanoic moieties of said ester have from 5 to 25 carbon atoms and wherein said alkanopolyol has from 2 to 6 carbon atoms and from 2 to 4 alcoholic hydroxyl groups.

8. A process which comprises contacting a dialkanoic diester of a polyoxyalkylene glycol with from 0.05 to 1.0 weight percent of urea, based on weight of said diester, at a temperature in the range of from 125° C. to 250° C. for a period of from 10 to 60 minutes, and thereafter recovering the said diester having reduced corrosive tendencies to metals thus produced, wherein the alkanoic moieties of said diester have from 5 to 25 carbon atoms and wherein the oxyalkylene moieties of said polyoxyalkylene glycol have from 2 to 3 carbon atoms.

9. A process which comprises contacting a monoalkyl ether of a polyoxyalkylene glycol with from 0.05 to 1.0 weight percent of urea, based on weight of said ether, at a temperature of from 125° C. to 250° C. for a period of from 10 to 60 minutes, and thereafter recovering the said ether having reduced corrosive tendencies to metals thus produced, wherein the alkyl moiety of said ether has from 1 to 12 carbon atoms and wherein the oxyalkylene moieties of said ether have from 2 to 3 carbon atoms.

10. The process of claim 5 wherein said dialkyl diester of an alkanedioic acid is 2-ethylhexyl isodecyl azelate.

11. The process of claim 5 wherein said dialkyl diester of an alkanedioic acid is di(2-ethylhexyl) adipate.

12. The process of claim 5 wherein said dialkyl diester of an alkanedioic acid is diisodecyl adipate.

13. The process of claim 9 wherein the monoalkyl ether of a polyoxyalkylene glycol is polyoxypropylene glycol monobutyl ether.

14. The product obtained by the process of claim 1.

15. The product produced by the process of claim 4.

16. The product produced by the process of claim 5.

17. The product produced by the process of claim 9.

#### References Cited in the file of this patent

#### UNITED STATES PATENTS

|           |                          |               |
|-----------|--------------------------|---------------|
| 2,224,158 | Marks et al. -----       | Dec. 10, 1940 |
| 2,408,090 | Musher -----             | Sep. 24, 1946 |
| 2,599,736 | Adelson et al. -----     | June 10, 1952 |
| 2,657,984 | Braithwaite et al. ----- | Nov. 3, 1953  |
| 2,727,025 | Weitkamp -----           | Dec. 13, 1955 |
| 2,908,647 | Vaughn -----             | Oct. 13, 1959 |
| 2,929,786 | Young et al. -----       | Mar. 22, 1960 |
| 2,944,973 | Langer et al. -----      | July 12, 1960 |
| 3,044,949 | Schlenk -----            | July 17, 1962 |

#### OTHER REFERENCES

25 McTurk, "Synthetic Lubricants," USAF Wright Air Development Center Technical Report 53-88 (Oct. 1953). Printed by McGregor & Werner, Inc., Dayton, Ohio (March 1954). Pages 20-21, 33-34, 43-44 pertinent.